

# UNITED STATES PATENT OFFICE.

WILLIAM B. ALLMAN, OF INDIANAPOLIS, INDIANA.

## ROOFING COMPOSITION.

SPECIFICATION forming part of Letters Patent No. 246,359, dated August 30, 1881.

Application filed February 14, 1881. (No specimens.)

*To all whom it may concern:*

Be it known that I, WILLIAM B. ALLMAN, a citizen of the United States, residing at Indianapolis, in the county of Marion and State 5 of Indiana, have invented a new and useful Composition of Matter to be used for Roofing, of which the following is a specification.

My composition consists of the following ingredients, combined in about the proportions 10 stated, viz: Common coal-tar, seventy-five pounds; pitch, twenty-five pounds; ground slate, three hundred pounds; plasterers' hair, ten pounds. These ingredients are thoroughly mixed in the following manner, to wit: The 15 coal-tar and pitch are melted together in an iron tank or kettle surrounded with boiling water in another kettle or tank, until they are well mixed and become perfectly liquid; then the slate-flour is thoroughly mingled by agitation therewith until the mass becomes too thick to run; then the hair is stirred into the mass, and the whole is thoroughly mixed.

In putting on roofing of the above-described composition I prefer to use Manila cloth as 25 the base, which is tacked or otherwise secured to the roof-sheeting, and the composition is applied to the manila at a boiling temperature, which, upon cooling, forms an even coat-

ing, which is elastic, and not liable to crack or run, even on steep roofs, and is fire-proof. The 30 plasterers' hair adds greatly to its strength and durability by preventing the compound from cracking. The pitch and tar unite to form a body which absorbs large quantities of the slate-flour. The pitch gives elasticity to 35 the mass, and the slate-flour effectually destroys the combustible nature of the compound and renders the roofing fire-proof.

What I claim as new, and desire to secure 40 by Letters Patent, is—

The herein-described composition of matter to be used for roofing purposes, consisting of common coal-tar, pitch, slate-flour, and plasterers' hair, in about the proportions specified, the coal-tar and pitch being first melted and 45 mixed, then the slate-flour and plasterers' hair are added, and the whole mass thoroughly mixed, substantially as described.

In testimony whereof I have signed my name to this specification in the presence of two sub- 50 scribing witnesses.

WILLIAM B. ALLMAN.

Witnesses:

E. O. FRINK,  
G. H. RENNETT.